# EUROPEAN PATENT SPECIFICATION

(11) **EP 0 249 973 B1**
(45) Date of publication and mention of the grant of the patent: **06.11.1991**
(21) Application number: 87108724.3
(22) Date of filing: 16.06.1987
(51) Int. Cl.: H01F 1/08

(54) **Permanent magnetic material and method for producing the same**
Dauermagnet-Material und Verfahren zur Herstellung
Matériel d'aimant permanent et procédé pour produire celui-ci

(30) Priority: 16.06.1986 JP 139650/86; 11.04.1987 JP 89028/87
(43) Date of publication of application: 23.12.1987
(73) Proprietor: TOKIN CORPORATION, Sendai-shi Miyagi-ken (JP)
(72) Inventor: Sasaki, Kinya, Sendai-shi Miyagi-ken (JP); Otsuki, Etsuo, Sendai-shi Miyagi-ken (JP); Otsuka, Tsutomu, Sendai-shi Miyagi-ken (JP); Fujiwara, Teruhiko, Sendai-shi Miyagi-ken (JP)
(74) Representative: Prüfer, Lutz H., Dipl.-Phys.

(56) References cited:
- EP-A- 0 166 597
- IEEE TRANSACTIONS ON MAGNETICS; vol. MAG-8, no. 3, September 1972, Kyoto, Japan KARL J. STRNAT "The Hard-Magnetic Properties of Rare Earth-Transition Metal Alloys" pages 511-516
- APPLIED PHYSICS LETTERS, vol. 39, no. 10, November 15, 1981, Washington D.C. N.C. KOON, B.N. DAS "Magnetic properties of amorphous and crystallized (Fe0, 82B0,18)0,9 Tb0, 5La0, 05" pages 840-842
- JOURNAL OF APPLIED PHYSICS, vol. 55, no. 6, part IIA, March 15, 1984, Michigan J.J. CROAT et al. "Pr-Fe and Nd-Fe-based materials: A new class of high-performance permanent magnets" pages 2078-2082

## Description

### 1) Field of the Invention

This invention relates to a permanent magnet material of a bulk shape and, in particular, to an iron-rare earth metal-boron (R-Fe-B) permanent magnet material with a high coercive force.

### 2) Description of the Prior Art

Permanent magnets have been used in various applications such as electromechanical apparatus.

Recently, demands for Sm-Co permanent magnets have increased in place of known alnico magnets, ferrite magnets, and other conventional magnets, because of the high energy product of Sm-Co magnets. However, the Sm-Co magnets are expensive because of use of cobalt.

Therefore, various approaches are made for new permanent magnets which are economical and have an increased energy product.

A possible approach has been directed to a novel intermetallic compound of transition metal (T) and rare earth metal (R) instead of the Sm-Co intermetallic compound.

However, the intermetallic compounds without use of Co have been considered impossible to produce a magnet having coercivity which is associated with magnetocrystalline anisotropy because the compounds have an easy magnetization direction in the crystal phase. A reference is made to K. J. Strnat; IEEE Trans. Mag. (1972) 511.

In Appl. Phys. Lett. 39(10) (1981), 840, N. C. Koon and B. N. Das disclosed magnetic properties of amorphous and crystallized alloy of (Fe₀_{.82}B₀_{.18})₀_{.9}Tb_{0.05}La₀_{.05}. They wrote that crystallization of the alloy occurred near the relatively high temperature of 900 K, which also marked the onset of dramatic increase in the intrinsic coercive force. They found out that the alloy in the crystallized state appeared potentially useful as low cobalt permanent magnets.

It is considered that magnetically hard intermetallic compound of R-Fe-B (R = Tb and La) are formed in the alloy. Reviewing the R-Fe-B (R=Gd, Sn, Nd) ternary phase diagram by N. F. Chaban, Y. B. Kuz'ma, N. S. Bilonizhko, O. O. Kachmar and N. W. petriv; Dopodivi Akad. Nuk. Ukr. RSR, Ser. A (1979) No.10, P.P. 875-877, the intermetallic compound R-Fe-B (R = Tb and La) by Koon et al is guessed to be represented by R₃Fe₁₆B, which is confirmed to be Nd₂Fe₁₄B by J. J. Croat et al. Reference is made to J. J. Croat, J. F. Herbst, R. W. Lee and F. E. Pinkerton; J. Appl. Phys, 55 (1984) 2078.

Therefore, considering the saturation magnetization of an intermetallic compound of R-T as shown in the above-described reference by K. J. Strnat, it can be guessed that use of Ce, Pr, and/or Nd for R in Fe-B-R alloy can provide better magnetic properties for permanent magnets than the Fe-B-La-Tb alloy.

J. J. Croat proposed amorphous (Nd and/or Pr)-Fe-B alloy having magnetic properties for a permanent magnet as disclosed in JP-A-60009852. Those magnetic properties were considered to be caused by a microstructure where Nd₂Fe₁₄B particles having a perticle size of 20-30 nm were dispersed within an amorphous Fe phase. Reference is further made to R. K. Mishra: J. Magnetism and Magnetic Materials 54-57 (1986) 450.

However, the amorphous alloy can provide only an isotropic magnet because of its crystallographically isotropy. This means that a high performance permanent magnet cannot be obtained from the amorphous alloy.

Sagawa, Fujiwara, and Matsuura proposed an anisotropic R-Fe-B sintered magnet in JP-A-59046008 which was produced from an ingot of an alloy of R (especially Nd), Fe, and B by conventional powder metallurgical processes. The sintered magnet has more excellent magnetic properties for permanent magnets than the known Sm-Co magnets.

However, the R-Fe-B sintered magnet has a problem in considerably low corrosion resistance.

Further, since the R-Fe-B alloy out of stoichiometric compound of Nd₂Fe₁₄B is active to oxygen, any care is necessary so as to prevent the alloy from oxidation. Moreover a surface oxide layer must be machined away after sintering process. Therefore, the magnet cannot be produced with a high dimensional accuracy.

It is an object of the present invention to provide a permanent magnet material of a bulk shape comprising R₂T₁₄B magnetic compound and having an excellent corrosion resistance.

It is another object of the present invention to provide a method for producing the bulk-shape permanent magnet material comprising R₂T₁₄B magnetic compound and having an excellent corrosion resistance.

It is still another object of the present invention to provide a method for producing the bulk-shape permanent magnet material comprising R₂T₁₄B magnetic compound with an excellent dimensional accuracy.

According to the present invention, a magnetic body with a high coercive force for a permanent magnet can be obtained which consists essentially of a metallic cementing phase and magnetic crystalline particles uniformly dispersed within the metal cementing phase. The cementing phase is 10% or less by volume of the magnetic body and comprises at least one element selected from a first metallic group of Al, Zn, Sn, Cu, Pb, S, In, Ga, Ge, and Te. The magnetic crystalline particles is substantially balance of the volume of the magnetic body and is a composition represented by a chemical formula R₂T₁₄B, where R is at least one element selected from Y and rare earth metals, T being transition metals and comprising Fe 50-100 at% in the transition metals. Each of the magnetic particles is embedded in the cementing phase to form an interface therebetween.

The cementing phase is inert to oxygen in comparison with Nd and has, therefore, a good corrosion resistance.

The cementing phase may comprise an intermetallic compound of at least one of the first metallic group and at least one selected from a second metallic group of R, T, and B.

The present invention further provides a method for producing a magnetic body with a high coercive force for a permanent magnet. The method comprises steps of: preparing an ingot of R-T-B magnetic alloy comprising a magnetic intermetallic compound represented by a chemical formula of R₂T₁₄B, where R is at least one element selected from Y and rare earth metals, T being transition metals but comprising Fe 50-100 at% in the transition metals; pulverizing and milling the ingot to thereby prepare a magnetic powder; preparing a metallic cementing powder comprising at least one element selected from a first metallic group of Al, Zn, Sn, Cu, Pb, S, In, Ga, Ge, and Te; mixing the metallic cementing powder of 10% or less by volume and the magnetic powder of substantially balance to prepare a mixed powder; and forming a bulk-shape body of the mixed powder at an elevated temperature.

The bulk-shape body forming step comprises steps of; compacting the mixed powder under influence of a grain aligning magnetic field into a compact body of a predetermined shape; and sintering the compact body at a temperature lower than a peritectic reaction temperature of the magnetic powder but higher than a melting temperature of the metallic cementing powder to thereby produce, as the bulk-shape body, a sintered body.

The sintered body may be subjected to a heat treatment at a temperature, preferably, 300-900 °C for improving the magnetic properties of the sintered body.

The bulk-shape body forming step may be hot compaction process for hot compacting the mixed powder into the bulk-shape body at an elevated temperature lower than 1,100 °C but higher than a melting temperature of the metallic cementing powder.

The hot compaction process is a hot-pressing process and alternatively a hot-extrusion process.
Fig. 1 is a schematic view of a microstructure of a bulk-form permanent magnet material according to the present invention;
Fig. 2 is a view illustrating variation of magnetic properties of a magnet to a volume percent of to Nd₃₀Fe₄₀Al₃₀ in the magnet;
Fig. 3 is a view illustrating a microstructure of a permanent magnet material of (Nd₂Fe₁₄B)₉₅(Nd₃₀Fe₄₀Al₃₀)₅ according to an example of the present invention;
Fig. 4 is a view illustrating a microstructure of a permanent magnet material of (Nd₂Fe₁₄B)₈₉_{.5}(NdCu₂)₁₀_{.5} according to another example of the present invention;
Fig. 5 is a view illustrating a microstructure of a permanent magnet material of (Nd₂Fe₁₄B)₉₅(Pb₆₉_{.6}Sn₃₀_{.4})₅ according to still another example of the present invention;
Fig. 6 is a view illustrating a microstructure of a permanent magnet material of (Nd₂Fe₁₄B)₉₅(Nd₄₀Fe₂₀Pb₂₀Sn₂₀)₅ according to yet another example of the present invention;
Fig. 7 is a view illustrating variation of a coercive force of a permanent magnet material in an example to a heat treatment temperature; and
Fig. 8 is a view illustrating variation of a coercive force of a permanent magnet material in an example to a heat treatment time period.

The present invention attempts to provide a permanent magnet material with a high coercive force and a corrosion resistance by making the material to have a microstructure as shown in Fig. 1 where magnetic particles of stoichiometric intermetallic compound of Nd₂Fe₁₄B are dispersed within a metallic cementing phase. The metallic cementing phase is composed of metallic elements and/or an intermetallic compound or compounds, which are inert to oxygen in comparison with Nd.

In order to realize the microstructure, Nd₂Fe₁₄B powder and metallic cementing powder are separately prepared and those powder are mixed. The mixed powder is sintered or hot-formed at an elevated temperature into a bulk-shape body so that the cementing powder forms a cementing phase to cement the magnetic particles together.

The metallic element or elements are selected to be ones each having a melting point lower than a peritectic temperature of the intermetallic compound of Nd₂Fe₁₄B, and the elevated temperature is also selected lower than the peritectic temperature but higher than the melting point of the cementing powder. Therefore, only the cementing powder melts to form the cementing phase by the sintering process or hot compaction process while the intermetallic compound of the magnetic powder is not melted but dispersed within the cementing phase.

Nd is active to oxygen if they do not form any intermetallic compound together or with other metallic element or elements. Therefore, it is desired that the cementing phase includes no Nd.

However, at the high temperature for the sintering or hot-compaction, Nd and/or Fe diffuse from the magnetic powder into the cementing phase so that the intermetallic compound of Nd₂Fe₁₄B is decomposed. In order to prevent the intermetallic compound of each magnetic particle from decomposition, Nd and Fe are included in the cementing powder in the form of an intermetallic compound or compounds with other metallic element or elements. Alternatively, the magnetic powder is prepared as an alloy powder including Nd and Fe in addition to the intermetallic compound of Nd₂Fe₁₄B.

In either use of the former and the latter ways, Nd and Fe are present in the cementing phase of the produced body. However, Nd forms an intermetallic compound with the other metallic element or elements. Accordingly, the cementing phase is also excellent in corrosion resistance.

Generally speaking, since a comparatively high temperature is used in the sintering temperature, both of the former and the latter can be employed. However, since a comparatively low temperature is used in the hot compaction process, the latter is employed because intermetallic compound of Nd and Fe with the other metallic element is apt to have a melting temperature higher than the temperature for hot compaction.

The amount of the cementing powder is limited at maximum 10 % by volume of the mixed powder, because when the cementing powder exceeds 10 vol%, the amount of the magnetic powder is insufficient to obtain a high remanence.

It should be noted that the intermetallic compound of Nd₂Fe₁₄B has a high residual magnetic flux density but has not a coercive force sufficient for a permanent magnet.

Now, the present invention will be described in connection with examples.

### Example 1

An ingot of an intermetallic magnetic alloy represented by Nd₁₃Fe₈₁B₆ was prepared by the induction melting in argon gas atmosphere. Purity factors of used start materials of Nd, Fe (electrolytic iron), and B were 98%, 99.9%, and 99.5% or more, respectively. The ingot was pulverized by a crusher to have a particle size below 24 mesh (Tyler) and, thereafter, finely divided by a ball mill into a fine magnetic powder having an average particle size of 3 µm.

On the other hand, various metallic powders (Zn, Al, S, In, Ga, Ge, Sn, Te, Cu, and Pb) for the cementing phase material were prepared, each powder having an average particle size of several tens micron meters and a purity of 99.9% or more.

Each metallic powder was mixed with the fine magnetic powder to form mixed powder. Each metal was adjusted at 58 by volume of the mixed powder. Zn, Al, S, In, Ga, Ge, Sn, Te, Cu, and Pb were, by weight, 5%, 2%, 2%, 5%, 4%, 4%, 5%, 4%, 6%, and 7% in the mixed powders, respectively.

After being mixed in a ball mill, each mixed powder was hot-pressed into a desired bulk-shape body under a pressing stress of 1,000 Kg.f/cm² at a temperature of 600°C within argon gas atmosphere for 15 minutes.

Each hot-pressed body was measured as to density d, residual magnetic flux density Br, coercive force _{I}H_{C}, maximum energy product (BH)max. The measured data are demonstrated with sample numbers 1-10 in Table 1.

As a comparative sample, starting materials of Nd, Fe, B, and Al were blended with each other to obtain an alloy represented by (Nd₁₅Fe₇₇B₇)₉₅Al₅ and an ingot of the alloy was produced by use of an induction furnace. The ingot was finely ground into a fine powder, which was, in turn, hot-pressed into a desired bulk-shape body under similar conditions as described above. While, an ingot represented by Nd₁₃fe₈₁B₆ was prepared in the similar manner and a hot-pressed body was produced from the ingot under the similar manner as described above. Densities and magnetic properties of those two hot-pressed bodies are shown with sample numbers 11 and 12, respectively, in Table 1.

Table 1 teaches that the samples Nos. 1-10 according to an embodiment of this invention are superior to comparing samples Nos. 11 and 12 according to the known production method in the magnetic properties, especially, the maximum energy product (BH)max.

### Example 2

A fine magnetic powder of Nd₁₃Fe₈₁B₆ was prepared and was mixed with metal powders (each having an average particle size of 20-30 um ) of Zn 5wt%, Al 2wt%, S 2wt%, In 5wt%, Ga 4wt%, Ge 4wt%, Sn 5wt%, Te 4wt%, Cu 6wt%, and Pb 7wt%, respectively, in the similar manner as described in Example 1.

Each mixed powder was compacted into a compact body of a desired bulk-shape by application of a pressing force of 1.5 ton.f/cm² under influence of a grain aligning magnetic field of 25 KOe. The compact body was hot-pressed at 600°C by pressing stress of 1,000 Kg.f/cm² within vacuum for 15 minutes. Each hot-pressed body was subjected to measurement of density and magnetic properties. The measured data are shown as sample Nos. 13-22 in table 2.

For comparing with these samples, alloy ingots of (Nd₁₅Fe₇₇B₇)₉₅Al₅ and Nd₁₄Fe₈₁B₆ were produced and were finely ground into powders. Those powders were compacted into compact bodies of a desired bulk shape and were hot-pressed in the similar manner. Densities and magnetic properties of those hot-pressed bodies are shown as sample Nos. 23 and 24 in Table 2.

It should be noted from Table 2 that sample Nos. 13-22 according to embodiments of the present invention are superior in the magnetic properties to not only comparing samples of Nos 23 and 24 according to the known producing method but also samples of Nos. 1-10 in Table 1 according to embodiments of the present invention.

### Example 3

In the similar manner as described in Example 1, Nd₂Fe₁₄B magnetic alloy ingot was prepared and was pulverized to have a particle size below 24 mesh (Tyler).

While, for the cementing phase material, start materials of Nd (having a purity factor of 98% or more), Fe (having a purity factor of 99.9% or more), and Al (having a purity factor of 99.9%) were mixed and melted by the induction melting in argon gas atmosphere to form an ingot of Nd₃₀Fe₄₀Al₃₀ alloy. The ingot was also pulverized into powder having a particle size below 24 (Tyler) mesh.

Both of the powders were blended with each other at various mixing ratios so that Nd₃₀Fe₄₀Al₃₀ powder is 0-15% by volume of the blended powder.

Each blended powder was finely ground into a powder of an average particle size of about 4 µm. The finely ground powder was compacted into a compact body of a desired bulk-shape by application compacting stress of 1.5 ton.f/cm² under influence of a grain aligning magnetic field of 20 KOe. The compact body was sintered in vacuum at 1,000-1,150 °C for 2 hours. The sintered body was heat treated at 500-900 °C for one hour. Density d, residual magnetic flux density Br, coercive force _{I}H_{C}, and (BH)max of the sintered body after heat treatment were measured are are illustrated in Fig. 2 for various volume percents of Nd₃₀Fe₄₀Al₃₀ in the sintered body.

In Fig. 2, the maximum magnetic properties are obtained at 5 vol% of Nd₃₀Fe₄₀Al₃₀ content. The magnetic properties are shown as a sample No. 25 in Table 3. The table also has properties of a comparing sample No. 26 which was a sintered Nd₁₄Fe₈₀B₆ alloy produced from the alloy ingot through milling, compacting in the aligning magnetic field, sintering, and heat treating steps according to a conventional powder metallurgy.

It will be understood from Table 3 that sample No.25 according to the present invention has a considerably excellent magnetic properties in comparison with sample No. 26 according to the conventional process.

The sintered body of sample No. 25 was cross-sectioned and polished. The microstructure in the polished surface was observed by a Scanning Electron Microscope (SEM). The observed microstructure is illustrated in Fig. 3.

Referring to Fig. 3, it will be noted that the magnetic crystalline particles (being black) of Nd₂Fe₁₄B are covered with, or embedded in, a cementing phase (being white) of Nd₃₀Fe₄₀Al₃₀.

Then, the No.25 sample was subjected to component analysis of the magnetic particles and the cemented phase in the sample by use of an Electron Probe Micro Analyser (EPMA). Analysed elements and their amount (at%) are shown in Table 4.

This example teaches us that magnetic properties of sintered Nd₂Fe₁₄B magnet can be considerably improved by covering and cementing the Nd₂Fe₁₄B particles with the Nd(Fe, Al)₃ matrix or the cementing phase.

Fig. 2 shows that the magnetic properties gradually decrease along increase of the cementing phase from 5 vol% through 8 vol%. It is considered that this is because of decrease of the amount of the magnetic particles.

### Example 4

Nd₂Fe₁₄B alloy powder and Nd₃₀Fe₄₀Al₃₀ alloy powder produced through the similar steps as described in Example 3 were blended with each other so that Nd₃₀Fe₄₀Al₃₀ powder was 5% of volume of the blended powder. The blended powder was compacted to a desired bulk shape in the grain aligning magnetic field of 20 KOe by application of compacting force of 1.5 ton.f/cm² and produced a green compact body. The green compact body was subjected to a hot compaction by hot-pressing the green compact at 800 °C in argon gas atmosphere by 1,000 Kg.f/cm² for 15 minutes.

Density and magnetic properties of the hot-pressed body were measured and are described with sample number of No. 27 in Table 5.

In Table 5, sample No. 28 is a sample produced from a Nd₁₄Fe₈₀B₆ powder through the similar compacting and hot-pressing steps.

Comparison of sample Nos. 27 and 28 also teach that the Nd-Fe-Al cementing phase improves the magnetic properties of Nd₂Fe₁₄B magnet.

### Example 5

Nd₂Fe₁₄B magnetic alloy powder with an average particle size of 3 µm was prepared in the similar manner as described in Example 1. While, NdCu₂ powder for the cementing phase material having similar particle size was also produced in a similar producing method. Both powders were mixed with each other so that the amount of NdCu₂ powder was about 10% by volume in the mixture, and the mixture was uniformly mixed in a ball mill. The mixture was compacted into a bulk shape by application of compacting stress of 1.5 ton.f/cm² in the grain aligning magnetic field of 20 KOe. The compacted body was sintered in vacuum at 1,100-1,130 °C for 2 hours. The sintered body was heat-treated in argon gas atmosphere at 600-800 °C for one hour.

The magnetic properties of the sintered body as sample No. 29 are shown in Table 6 together with its density.

No. 29 sample was then cross-sectioned and polished. The microstructure of the cross-section was observed by use of an optical microscope. The observed microstructure is illustrated in Fig. 4. In the figure, Nd₂Fe₁₄B magnetic particle is shown in white and the NdCu₂ cementing phase is shown in black.

Further, the electron beam X-ray microanalysis was carried out to the magnetic particle phase and the cementing phase of the sample of No. 29. Table 7 shows analysed elements and their amounts by atomic percent (at%).

In Table 7, the cementing phase comprises two intermetallic compounds I and II. Compound I is represented by NdCu, and Compound II is represented by Nd(Cu, Fe)₂.

As being illustrated in Fig. 4, each magnetic particle (shown in white in Fig. 4) is cemented and covered with the cementing phase (black in Fig. 4).

### Example 6

A mixture similar to in Example 5 was prepared.

The mixture was hot-pressed in argon gas atmosphere at 900 °C by application of pressing stress of 1,000 Kg.f/cm² for 15 minutes.

Table 8 shows density and magnetic properties of the hot-pressed body as sample No. 30. Table 8 teaches us that excellent magnetic properties are obtained.

### Example 7

Nd₂Fe₁₄B magnetic powder similar to Example 5 was prepared. While, Nd₂₅_{.4}Cu₅₂_{.2}Zn₂₂_{.4} powder for the cementing phase was prepared in the similar manner as the magnetic powder. Both of the powders were blended with each other so that the amount of the Nd₂₅_{.4}Cu₅₂_{.2}Zn₂₂_{.4} powder was about 10% by volume of the blended powder. The blended powder was uniformly mixed in ball mill. The mixture was hot-pressed into a body of a desired shape in argon gas at 600 °C by pressing stress of 1,000 Kg.f/cm² for 15 minutes.

The magnetic properties and density of the hot-pressed body are shown in Table 9.

### Example 8

A molten alloy of Nd₃₄Fe₆₅B was prepared in the similar way as in Example 1.

While, two Pb-Sn alloys A and B shown in Table 10 were also prepared in the molten state by using start materials of Pb and Sn each having purity factor of 99.9% or more.

A powder less than 250 (Tyler) mesh was prepared from each of the molten alloys by atomization. Then, Nd₁₆Fe₁₈B₆ magnetic powder was divided by ball mill into average particle size of about 3 µm. Each powder of Pb-Sn alloys A and B was blended with the magnetic powder and was mixed in ball mill. The amount of each of alloy A and B was 5% by volume of each mixture.

Each powder mixture was compacted into a compact body of a bulk shape in the aligning magnetic field of 20 KOe by compacting stress of 1.5 ton.f/cm². The compact body was sintered in vacuum at 1,000-1,150 °C for 2 hours. The sintered body was heat-treated at 500-900 °C for one hour and was thereafter subjected to measurement of density and magnetic properties.

The measured data are demonstrated in Table 11. No. 32 sample uses alloy A and No. 33 uses alloy B.

The microstructure of each sample of Nos. 32 and 33 was observed by an optical microscope. Fig. 5 shows the microstructure of No. 32 sample. In the figure, the magnetic particles are illustrated in white and the cementing phase is black.

While, the microanalysis was performed to the magnetic perticle phase and the cementing phase of each sample of Nos. 32 and 33. The analysed elements are shown in Table 12 together with their amounts by at%.

Attention should be directed to a fact that the magnetic particle phase consists of the intermetallic compound of Nd₂Fe₁₄B. While, Nd and Fe is present in both of the cementing phase. I and II are analysed data at different portions of the cementing phase of the sintered body.

For sample No. 33, it will be appreciated that the cementing phase is constituted of an intermetallic compound of Nd(Pb, Fe, Sn) where a part of Pb in NdPb is replaced by Fe and Sn. While, the cementing phase in No. 33 sample is composed of an intermetallic compound of Nd(Sn, Fe, Pb) where a part of Sn in NdSn compound is replaced by Fe and Pb.

That is, Nd and Fe diffuse from Nd-Fe-B particles into Pb-Sn phase so that each Nd-Fe-B particle becomes a stoichiometric intermetallic compound R₂Fe₁₄B which has ferromagnetism.

If Nd and Fe are insufficiently diffused in the Pb-Sn alloy, excellent magnetic properties are not obtained because each magnetic particle comprises not only the intermetallic compound of Nd₂Fe₁₄B but also non-magnetic phase.

This means that it is useful for production of the permanent magnet material to prepare Nd₂Fe₁₄B particles and to mix the particles with cementing phase materials so as to obtain a bulk-shape magnet material having excellent magnetic properties.

### Example 9

The powder mixtures prepared in Example 8 were compacted into green compact bodies in the aligning magnetic field of 20 KOe by compacting stress of 1.5 ton.f/cm². Each green compact body was hot-pressed in argon gas at 750 °C under application of a pressure 1,000 Kg.f/cm² for 20 minutes. Thereafter, the hot-pressed body was heat-treated in argon gas at 600 °C for 30 minutes.

The magnetic properties after the heat treatment are shown in Table 13. Samples of Nos. 34 and 35 in Table 13 contain the Pb-Sn alloys A and B in Table 10, respectively.

In this embodiment, it was also confirmed that Nd and Fe were present in the cementing phase with the particles becoming Nd₂Fe₁₄B compound.

### Example 10

Nd₂Fe₁₄B magnetic alloy powder similar to Example 3 was prepared.

In the similar producing steps, Nd-Fe-Pb-Sn alloy powders C, D, and E in Table 14 were produced from

start materials of Nd (purity of 98 % or more), Fe (purity of 99.9% or more), Pb (purity of 99.9%), and Sn (purity of 99.9%). Each powder of C-E was prepared to have an average particle size of 3 µm.

These powders C-E were blended with the magnetic powder, separately, and each blended powder was mixed with each other in a ball mill. Each alloy powder of C-E was 5% by volume of each powder mixture.

Each powder mixture was compacted into a compact body in the aligning magnetic field of 20 KOe by compacting force of 1.5 ton.f/cm², and the compact body was sintered in vacuum at 1,000-1,150 °C for 2 hours. The sintered body was further heat-treated at 500-900 °C.

Table 15 indicates density and magnetic properties of each sintered and heat-treated body as samples Nos. 36, 37, and 38 which use Nd-Fe-Pb-Sn alloys C, D, and E, respectively.

In comparison with Nos. 32 and 33 samples, Nos. 36-38 samples are nearly equal to them in the magnetic properties but have a reduced Nd content which is active to oxygen. Accordingly, Nos. 36-38 samples are superior to Nos. 32 and 33 samples in the corrosion resistance and especially during production and storage of powder materials.

For each sintered body, the observation of microstructure and microanalysis were carried out. The microstructure of No. 38 sample is shown in Fig. 6 (white for magnetic particles and black for cementing phase), and analysed elements in respective samples are described in Table 16.

It will be understood from Table 16 that not only B but Nd and Fe do not diffuse into the Nd-Fe-Pb-Sn cementing phase. Pb and Sn nor diffuse into Nd₂Fe₁₄B particles.

### Example 11

Each mixture obtained in Example 10 was compacted into a green compact in the aligning magnetic field of 25 KOe by pressing stress of 1.5 ton.f/cm². The green compact was hot-pressed in argon gas at 800 °C by pressing stress of 1.0 ton.f/cm² for 20 minutes. Then, the hot-pressed body was heat-treated in argon gas atmosphere at 600 °C for 30 minutes.

Table 17 shows density and magnetic properties of each hot-pressed body after heat-treated as samples Nos. 39, 40, and 41.

Nos. 39 and 40 samples have magnetic properties equally to Nos. 34 and 35 samples but have a reduced amount of Nd.

Next, in order to appreciate of corrosion resistance of permanent magnet material according to the present invention, samples of Nos. 25, 29, and 32 according to the present invention and No. 26 sample sintered by the conventional powder metallurgy were subjected to the following tests.

### Test 1

A humidity test was carried out onto the test pieces under a test condition of a temperature of 60 °C and a humidity of 90% for 100 hours.

The result of the test is shown in Table 18, which teaches us that the samples according to the present invention are superior in corrosion resistance to the sample according to the conventional powder metallurgy.

### Test 2

Test pieces of each sample were coated with surface coatings by electrolytic Ni plating, phosphate treating, and anti-corrosion resin coating, respectively.

The electrolytic Ni plating was carried out after Cu plating coating of 3-5 µm thickness was previously formed.

The phosphate treating was performed using a conventional phosphate solution.

In the anti-corrosion resin coating, epoxy resin was dissolved in an organic solvent and then sprayed onto test pieces. Thereafter, epoxy resin coating was formed by heating at 150 °C.

Those test pieces were subjected to salt spray corrosion test under a condition where salt water solution (5% NaCl) was sprayed onto the test pieces at 35 °C for 48 hours during which surface change of each test piece was observed. When the test completed, magnetic properties of each test were measured.

The observed surface change and the measured magnetic properties are illustrated in Tables 19 and 20.

It will be noted from Table 19 that permanent magnet materials according to the present invention are excellent in corrosion resistance. The magnetic properties are not degraded by anti-corrosion surface coating as well be understood from Table 20.

### Example 12

Zn, Sn, and Al powders, each having a purity factor of 99.9%, were blended with the Nd₁₃Fe₈₁B₆ magnetic alloy powder obtained in Example 2, respectively, and the blend was mixed uniformly in ball mills to obtain respective powder mixtures.

Added amounts of Zn, Sn, and Al powders were selected to be 5% by volume of respective powder mixtures.

Each powder mixture was compacted in the aligning magnetic field of 25 KOe by pressing stress of 1.5 ton.f/cm² and formed a green compact of a desired bulk shape. The green compact was heated at 700 °C and then coated with glass coating by depositing glass powder onto the surface of the green compact. The glass coated green compact was inserted in a extrusion mould and was moulded into a desired shape by extrusion.

Each extruded body was measured to obtain the magnetic properties. The measured properties and densities are indicated for Nos. 42, 43, and 44 samples in Table 21 together with density.

In Table 21, each of Nos. 45 and 46 samples is a hot-pressed body produced from the alloy ingot through pulverizing, compacting, and extruding steps.

Magnetic materials according to the present invention can be produced by hot extrusion and has excellent magnetic properties in comparison with one produced from the alloy ingot.

### Example 13

Each of green compact obtained in Example 12 was hot-pressed in argon gas atmosphere at 700 °C by pressing stress of 1,000 Kg.f/cm² for 15 minutes. The hot-pressed body was heat-treated in argon at 600 °C for 10 minutes.

Magnetic properties of each hot-pressed body as sample of Nos. 47, 48, and 49 were measured before and after the heat treatment and are illustrated in Table 22. It will be found out from Table 22 that the coercive force _{I}H_{c} is improved by the heat-treatment with the other properties being almost unchanged. The improvement is considered to be caused due to decrease of nucleation sites of reverse domain by the heat-treatment.

In order to confirm influence of heat-treating temperature for the improvement of coercive force, heat treatment was carried out to No. 47 sample at various temperatures. Fig. 7 illustrates measured coercive force to variation of heat-treating temperature. Fig. 7 shows that the effective temperature is 300-900 °C.

Further, experiment for heat-treatment was performed as to No. 47 sample at various heat-treating time periods at a constant temperature of 600 °C. Fig. 8 shows residual magnetic flux density Br and coercive force _{I}H_{C} to variation of heat-treating time period. It will be noted from Fig. 8 that the heat treatment for about 10 minutes is most effective for improvement of the magnetic properties.

### Example 14

Al₁₁Zn₈₉ powder and Al₈₃Cu₁₇ powder were produced from starting materials having purity of 98% or more. Each powder has an averaged particle size of 1-10 µm.

Each powder and the Nd₁₃Fe₈₁B₆ magnetic powder obtained in Example 2 were mixed with each other at a mixing ratio of 5 to 95 by volume (which means 4.4 wt% for Al₁₁Zn₈₉ and 2.4 wt% for Nd₁₃Fe₈₁B₆) in a ball mill.

The mixture was compacted to a green compact in the aligning magnetic field of 25 KOe by pressing stress of 1.5 ton.f/cm². The green compact was hot-pressed in argon gas atmosphere at 600 °C by pressing stress of 1,000 Kg.f/cm² for 15 minutes. The magnetic properties of hot-pressed body of sample Nos. 50 and 51 are described in Table 23.

It will be understood to obtain improvement of magnetic properties similar to Example 2.

### Example 15

Al₆₆Fe₃₄ powder, Al₂₅Ni₇₅ powder, Al₂₀Co₈₀ powder, and Al₇₅Cr₂₅ powder were used in place of Al₁₁Zn₈₉ powder and Al₈₃Cu₁₇ powder in Example 14, and a green compact was produced from a mixture of each powder and Nd₁₃Fe₈₁B₆ magnetic powder in similar manner as described in Example 14. The green compact was hot-pressed similarly, but for 10 minutes.

Magnetic properties of the hot-pressed body was excellent similarly as in Example 14 and is shown in Table 24 with sample numbers Nos. 52-55 for alloy powders used.

## Claims

1. A magnetic body with a high coercive force for a permanent magnet which consists essentially of a metallic cementing phase and magnetic crystalline particles uniformly dispersed within said metal cementing phase, said cementing phase being 10% or less by volume of said magnetic body and comprising at least one element selected from a first metallic group of Al, Zn, Sn, Cu, Pb, S, In, Ga, Ge, and Te, said magnetic crystalline particles being substantially balance of the volume of the magnetic body and being a composition represented by a chemical formula R₂T₁₄B, where R is at least one element selected from Y and rare earth metals, T being transition metals and comprising Fe 50-100 at% in the transition metal, each of said magnetic particles being embedded in said cementing phase to form an interface therebetween.

2. A magnetic body as claimed in Claim 1, said cementing phase comprising an intermetallic compound of at least one of said first metallic group and at least one selected from a second metallic group of R, T, and B.

3. A method for producing a magnetic body with a high coercive force for a permanent magnet comprising steps of:
preparing an ingot of R-T-B magnetic alloy comprising a magnetic intermetallic compound represented by a chemical formula of R₂T₁₄B, where R is at least one element selected from Y and rare earth metals, T being transition metal but comprising Fe 50-100 at% in the transition metal;
pulverizing and milling said ingot to thereby prepare a magnetic powder;
preparing a metallic cementing powder comprising at least one element selected from a first metallic group of Al, Zn, Sn, Cu, Pb, S, In, Ga, Ge, and Te;
mixing a metallic cementing powder of 10% or less by volume and said magnetic powder of substantially balance to prepare a mixed powder; and
forming a bulk-shape body of said mixed powder at an elevated temperature.

4. A method as claimed in Claim 3, said bulk-shape body forming step comprising;
compacting said mixed powder under influence of a grain aligning magnetic field into a compact body of a predetermined shape; and
sintering said compact body at a temperature lower than a peritectic reaction temperature of said magnetic powder but higher than a melting temperature of said metallic cementing powder to thereby produce, as said bulk-shape body, a sintered body.

5. A method as claimed in Claim 4, wherein said R-T-B ingot consists of said intermetallic compound of R₂T₁₄B, and said metallic cementing powder comprises an intermetallic compound of at least one element selected from said first metallic group and at least one selected from a second metallic group of R, T, and B.

6. A method as claimed in Claim 5, further comprising a step of subjecting said sintered body to a heat treatment for improving the magnetic properties of the sintered body.

7. A method as claimed in Claim 6, wherein said heat treatment is performed at 300-900 °C.

8. A method as claimed in Claim 3, wherein said bulk-shape body forming step is a hot compaction process for hot compacting said mixed powder into said bulk-shape body at an elevated temperature lower than 1,100 °C but higher than a melting temperature of said metallic cementing powder.

9. A method as claimed in Claim 8, wherein said hot compaction process is a hot pressing process for hot pressing said mixed powder into said bulk-shape body under a pressure of 5-5,000 Kg.f/cm².

10. A method as claimed in Claim 9, said bulk shape body forming step further comprising a step of previously compacting said mixed powder to form a green compact, said green compact being then subjected to said hot-pressing process.

11. A method as claimed in Claim 10, wherein said compacting step is performed within an aligning magnetic field.

12. A method as claimed in Claim 8, wherein said hot compaction process comprises steps of compacting said mixed powder to form a green compact, heating said green compact at said elevated temperature, and then subjecting said heated green compact to extrusion to thereby produce, as said bulk-shape body, an extruded body.

13. A method as claimed in Claim 12, wherein said green compact is coated with a heat insulating material prior to said extrusion.

14. A method as claimed in Claim 8, further comprising a step of subjecting said bulk-shape body to a heat treatment for improving the magnetic properties thereof.

15. A method as claimed in Claim 14, wherein said heat treatment is performed at 300-900 °C.

## Patentansprüche

1. Magnetischer Körper mit einer hohen Koerzitivkraft für einen Permanentmagneten, der im wesentlichen aus einer metallischen Zementphase und gleichmäßig in der metallischen Zementphase verteilten magnetischen kristallinen Teilchen besteht, wobei die Zementphase 10 % oder weniger im Volumen des magnetischen Körpers darstellt und mindestens ein Element aufweist, das aus einer ersten Metallgruppe aus Al, Zn, Sn, Cu, Pb, S, In, Ga, Ge und Te ausgewählt ist, die magnetischen kristallinen Teilchen das Volumen des magnetischen Körpers im wesentlichen ausgleichen und von einer Zusammensetzung sind, die durch eine chemische Formel R₂T₁₄B dargestellt ist, worin R ein aus Y und seltenen Erdmetallen ausgewähltes Element ist, T Übergangsmetalle sind und Fe bei 50 - 100 % in dem Übergangsmetall aufweisen und jedes der magnetischen Teilchen in der Zementphase zum Bilden einer Grenzfläche dazwischen eingebettet ist.

2. Magnetischer Körper nach Anspruch 1, wobei die Zementphase eine intermetallische Verbindung aus mindestens einem der ersten metallischen Gruppe und mindestens einem aus einer zweiten metallischen Gruppe aus R, T und B ausgewählten aufweist.

3. Verfahren zum Erzeugen eines magnetischen Körpers mit einer hohen Koerzitivkraft für einen Permanentmagneten mit den Schritten:
Vorbereiten eines Rohblockes aus einer R-T-B-Magnetlegierung, die eine magnetische intermetallische Verbindung aufweist, die durch eine chemische Formel R₂T₁₄B dargestellt wird, wobei R mindestens ein Element ist, das aus Y und seltenen Erdmetallen ausgewählt ist, B ein Übergangsmetall ist, aber Fe bei 50 - 100 % in dem Übergangsmetall aufweist;
Pulverisieren und Zermahlen des Rohbarrens zum dadurch Vorbereiten eines magnetischen Pulvers;
Vorbereiten eines metallischen Zementpulvers, das mindestens ein Element aufweist, das aus einer ersten Metallgruppe aus Al, Zn, Sn, Cu, Pb, S, In, Ga, Ge und Te ausgewählt ist;
Mischen eines metallischen Zementpulvers von 10 % oder weniger im Volumen und des magnetischen Pulvers zum im wesentlichen Ausgleichen zum Vorbereiten eines gemischten Pulvers und
Bilden eines bulkförmigen Körpers des gemischen Pulvers bei einer erhöhten Temperatur.

4. Verfahren nach Anspruch 3, wobei der Schritt des Bildens des bulkförmigen Körpers aufweist:
Verdichten des gemischten Pulvers unter Einfluß eines kornausrichtenden Magnetfeldes in einen verdichteten Körper einer vorbestimmten Form und
Sintern des verdichteten Körpers bei einer Temperatur, die niedriger ist als eine peritektische Reaktionstemperatur des magnetischen Pulvers, aber höher als eine Schmelztemperatur des metallischen Zementpulvers ist zum dadurch Erzeugen als der bulkförmige Körper eines gesinterten Körpers.

5. Verfahren nach Anspruch 4, bei dem der R-T-B-Rohbarren aus der intermetallischen Verbindung von R₂T₁₄B besteht und das metallische Zementpulver eine intermetallische Verbindung aus mindestens einem Element aufweist, das aus der ersten Metallgruppe gewählt ist, und eines, das aus einer zweiten Metallgruppe aus R, T und B ausgewählt ist.

6. Verfahren nach Anspruch 5, mit dem weiteren Schritt des Aussetzens des gesinterten Körpers einer Wärmebehandlung zum Verbessern der magnetischen Eigenschaften des gesinterten Körpers.

7. Verfahren nach Anspruch 6, bei dem die Wärmebehandlung bei 300 - 900 °C ausgeführt wird.

8. Verfahren nach Anspruch 3, bei dem der Schritt des Bildens des bulkförmigen Körpers ein warmer Verdichtungsvorgang zum warmen Verdichten des gemischten Pulvers in den bulkförmigen Körper bei einer erhöhten Temperatur niedriger als 1100 °C, aber höher als eine Schmelztemperatur des metallischen Zementpulvers ist.

9. Verfahren nach Anspruch 8, bei dem der warme Verdichtungsvorgang ein warmer Preßvorgang zum warm Pressen des gemischten Pulvers in den bulkförmigen Körper unter einem Druck von 5 - 5000 kp/cm² ist.

10. Verfahren nach Anspruch 9, wobei der Schritt des Bildens des bulkförmigen Körpers weiter einen Schritt des vorherigen Verdichtens des gemischten Pulvers zum Bilden eines Grünlings aufweist und der Grünling dann dem Warm-Pressen-Vorgang ausgesetzt wird.

11. Verfahren nach Anspruch 10, bei dem der Verdichtungsschritt in einem ausrichtenden Magnetfeld durchgeführt wird.

12. Verfahren nach Anspruch 8, bei dem der Warm-VerdichtungsVorgang die Schritte des Verdichtens des gemischten Pulvers zum Bilden eines Grünlings, Erwärmen des Grünlings bei der erhöhten Temperatur und dann Aussetzen des erwärmten Grünlings einem Extrudieren zum dadurch Erzeugen als dem bulkförmigen Körper eines extrudierten Körpers aufweist.

13. Verfahren nach Anspruch 12, bei dem der Grünling mit einem wärmeisolierenden Material vor dem Extrudieren beschichtet wird.

14. Verfahren nach Anspruch 8, das weiter einen Schritt des Unterwerfens des bulkförmigen Körpers einer Wärmebehandlung zum Verbessern seiner magnetischen Eigenschaften aufweist.

15. Verfahren nach Anspruch 14, bei dem die Wärmebehandlung bei 300 - 900 °C durchgeführt wird.

## Revendications

1. Corps magnétique à force coercitive élevée pour aimant permanent, constitué essentiellement d'une phase de cémentation métallique et de particules magnétiques cristallines uniformément dispersées dans la phase de cémentation métallique, cette phase de cémentation représentant 10 % au moins du volume du corps magnétique et comprenant au moins un élément choisi dans un premier groupe constitué des métaux Al, Zn, Sn, Cu, Pb, S, In, Ga, Ge et Te, les particules magnétiques cristallines représentant essentiellement le complément à 100 % du volume du corps magnétique et consistant en une composition représentée par une formule chimique R₂T₁₄B dans laquelle R est au moins un élément choisi dans des métaux Y et de terres rares, T étant constitué par des métaux de transition et comprenant de 50 à 100 % de Fe dans le métal de transition, chacune des particules magnétiques étant noyée dans la phase de cémentation pour former une interface entre elles.

2. Corps magnétique selon la revendication 1, caractérisé en ce que la phase de cémentation comprend un composé intermétallique constitué de l'un au moins des métaux du premier groupe et d'au moins un métal choisi dans un second groupe métallique de R, T et B.

3. Procédé de production d'un corps magnétique à force coercitive élevée pour aimant permanent, procédé caractérisé en ce qu'il comprend les différentes étapes consistant à :
préparer un lingot d'alliage magnétique de R-T-B comprenant un composé intermétallique représenté par formule chimique R₂T₁₄B dans laquelle R est au moins un élément choisi dans des métaux Y et de terres rares, T étant un métal de transition mais comprenant de 50 à 100 % de Fe dans le métal de transition ;
broyer et moudre le lingot pour préparer ainsi une poudre magnétique ;
préparer une poudre de cémentation métallique comprenant au moins un élément choisi dans un premier groupe constitué des métaux Al, Zn, Sn, Cu, Pb, S, In, Ga, Ge et Te ;
mélanger la poudre de cémentation métallique représentant 10 % ou moins du volume, avec la poudre magnétique représentant le complément à 100 % du volume, de manière à préparer une poudre mélangée ; et
former un corps en bloc de la poudre mélangée à une température élevée.

4. Procédé selon la revendication 3, caractérisé en ce que l'étape de formation du corps en bloc consiste à :
compacter la poudre mélangée sous l'influence d'un champ magnétique d'alignement des grains pour former un corps compact de forme prédéterminée ; et
fritter ce corps compact à une température inférieure à la température de réaction péritectique de la poudre magnétique mais supérieure à la température de fusion de la poudre de cémentation métallique pour produire ainsi, comme corps en bloc, un corps fritté.

5. Procédé selon la revendication 4, caractérisé en ce que le lingot de R-T-B est constitué du composé intermétallique de R₂T₁₄B, et en ce que la poudre de cémentation métallique comprend un composé intermétallique d'au moins un élément choisi dans le premier groupe de métaux et d'au moins un élément choisi dans le second groupe métallique de R, T et B.

6. Procédé selon la revendication 5, caractérisé en ce qu'il comprend en outre une étape consistant à soumettre le corps fritté à un traitement thermique pour améliorer les propriétés magnétiques de ce corps fritté.

7. Procédé selon la revendication 6, caractérisé en ce que le traitement thermique est effectué à 300-900°C.

8. Procédé selon la revendication 3, caractérisé en ce que l'étape de mise en forme du corps en bloc est un processus de compactage à chaud pour compacter à chaud la poudre mélangée de manière à former le corps en bloc à une température élevée inférieure à 1100°C, mais supérieure à la température de fusion de la poudre de cémentation métallique.

9. Procédé selon la revendication 8, caractérisé en ce que le processus de compactage à chaud est un processus de pressage à chaud pour presser à chaud la poudre mélangée de manière à former le corps en bloc sous une pression de 490.10³ à 490.10⁶ Pa (5 à 5000 Kg.f/cm²).

10. Procédé selon la revendication 9, caractérisé en ce que l'étape de formation du corps en bloc comprend en outre une étape consistant à compacter préalablement la poudre mélangée pour former un produit compact vert, ce produit compact vert étant ensuite soumis au processus de pressage à chaud.

11. Procédé selon la revendication 10, caractérisé en ce que l'étape de compactage est effectuée dans un champ magnétique d'alignement.

12. Procédé selon la revendication 8, caractérisé en ce que le processus de compactage à chaud comprend les étapes consistant à compacter la poudre mélangée pour former un produit compact vert, à chauffer ce produit compact vert à la température élevée, puis à soumettre le produit compact vert chauffé à une extrusion pour produire ainsi, comme corps en bloc, un corps extrudé.

13. Procédé selon la revendication 12, caractérisé en ce que le produit compact vert est recouvert d'un matériau d'isolation thermique avant l'extrusion.

14. Procédé selon la revendication 8, caractérisé en ce qu'il comprend en outre une étape consistant à soumettre le corps en bloc à un traitement thermique pour améliorer ses propriétés magnétiques.

15. Procédé selon la revendication 14, caractérisé en ce que le traitement thermique est effectué à 300-900°C.
